

## UNITED STATES PATENT OFFICE

WILLIAM TROTTER, OF NEW YORK, N. Y., ASSIGNOR TO MINERALS SEPARATION NORTH AMERICAN CORPORATION, OF NEW YORK, N. Y., A CORPORATION OF MARYLAND

## FROTH-FLOTATION CONCENTRATION OF ORES

No Drawing.

Application filed August 4, 1926. Serial No. 127,181.

This invention relates to the froth-flootation concentration of ores and is herein illustrated as applied to the concentration of ores whose principal value is carbonate of copper or carbonate of lead.

Such ores have hitherto proved refractory to treatment for concentration by the agents generally used when following the usual froth-flootation procedures.

10 Potassium and sodium xanthate have been extensively used in the froth-flootation concentration of sulphide ores, being usually used in the proportion of a tenth of a pound or less to a quarter of a pound per ton of ore. 15 Used in such proportions in the froth-flootation process they have markedly improved recoveries and have had other useful results. But these substances have been without substantial effect when used in these amounts in 20 attempting concentration of carbonate ores by the froth-flootation process.

According to the present invention these ordinary agents, as well as agents hitherto commercially untried, may be used according to modified procedures with the result that refractory ores like copper carbonate ores prove amenable to froth-flootation treatment in the machines hitherto used.

25 The invention is herein illustrated as carried out with the organic sulphur-containing compounds known as xanthates, mercaptides, and thio-phenol. It was also found possible to use para-thio-cresol, thio-beta naphthol, and mercapto-benzo-thiazole, these being progressively less effective. All the substances thus grouped contain simple sulphhydric radicals such as  $-S-H$ ,  $-S-Na$ ,  $-S-K$ , for example.

30 According to the present invention the xanthate and other substances are used in much larger amounts than has been customary in the froth-flootation process, with 35 the result that a copper carbonate ore is as effectively concentrated as is a sulphide ore. If only the organic sulphur-containing compounds are used in addition to the mineral-frothing agents, at least a pound, usually upwards of two pounds, per ton of ore of such

a substance, for example, a xanthate, has been used with a suitable mineral-frothing agent or agents to obtain commercial results.

Other features and advantages will hereinafter appear.

Example 1.—Suitably ground Bwana M'Kubwa copper ore containing 3.77% copper, the mineral being mainly carbonate of copper, was agitated in a five to one aqueous pulp with 0.32 pounds of pine oil and 4 pounds of potassium xanthate, both per ton of ore. A brilliant green froth float was obtained containing 10.44% copper and containing 94.1% of the copper in the ore. The froth was extremely stable, standing up several hours, dropping some gangue. The concentrates were capable of being easily re-cleaned.

Example 2.—A test similar except that only 2 pounds of the xanthate per ton of ore were used instead of the 4 pounds of Example 1, yielded a smaller float containing 10.02% copper and representing 79.2% of the copper in the ore.

Example 3.—Andes Copper Co. ore containing 1.19% copper largely in the form of copper carbonate, was agitated with a suitable mineral-frothing agent and with 4 pounds of potassium xanthate per ton of ore to yield a froth concentrate containing 9.5% copper and representing 51.1% of the copper in the ore.

Example 4.—Lead carbonate ore from the Shattuck-Arizona mine in Arizona, containing no identifiable sulphide, was agitated in a minerals separation subaeration machine for two minutes with 0.32 pounds of pine oil and one pound of potassium xanthate, both per ton of ore, and a first froth concentrate collected. There was then added two pounds more of the potassium xanthate, agitation continued for two minutes and a second froth concentrate collected. There was then added another two pounds of potassium xanthate and agitation continued for two minutes and a third froth concentrate collected. The mixed concentrates contained 27.10% of lead and contained 93.0% of the lead in the ore.

The detailed results are shown in the following table:

|               | Assays |       |       | Recoveries |
|---------------|--------|-------|-------|------------|
|               | Wt. %  | Pb. % | Pb. % |            |
| Heads.....    | 100.   | 4.3   | 100.  |            |
| 1st Conc..... | 9.9    | 30.   | 66.4  |            |
| 2nd Conc..... | 2.6    | 25.4  | 14.8  |            |
| 3rd Conc..... | 2.8    | 18.3  | 11.8  |            |
| Tails.....    | 84.7   | 0.37  | 7.0   |            |

*Example 5.*—An oxidized copper ore from the 3 R. mine at Patagonia, Arizona, was reground for fifteen minutes in a laboratory ball mill, made into a pulp with water, and agitated in a minerals separation spitzkasten subaeration testing machine for fifteen minutes with 0.6 pounds of crude pine oil, 4 pounds of potassium xanthate, and 0.3 pounds of steam distilled pine oil, all per ton of ore, to yield a rougher concentrate. This concentrate was reagitated for ten minutes with a further addition of 0.06 pounds of potassium xanthate per ton of ore to yield a finished concentrate and a middling. The results are shown in the following table:

|            | Assays |       |       | Recoveries |
|------------|--------|-------|-------|------------|
|            | Wt. %  | Cu. % | Cu. % |            |
| Heads..... | 100.   | 3.02  | 100.0 |            |
| Cone.....  | 10.9   | 25.20 | 90.7  |            |
| Midd.....  | 11.3   | 1.08  | 4.3   |            |
| Tails..... | 77.3   | .20   | 5.3   |            |

*Example 6.*—Bwana M'Kubwa ore ground to pass 65 mesh was made into a pulp with water and agitated for one minute in a subaeration testing machine with 4 pounds of potassium xanthate and 0.48 pounds of cresol, both per ton of ore, and then a froth concentrate removed for three minutes. There was then added a further 0.32 pounds of cresol per ton of ore, the pulp agitated for one minute, and then a second froth concentrate removed for three minutes. Finally there was further added 2 pounds of the xanthate and 0.4 pounds of cresol, both per ton of ore, the pulp agitated for one minute, and then a third froth concentrate removed for three minutes. The results are shown in the following table:

|               | Assays |       |       | Recoveries |
|---------------|--------|-------|-------|------------|
|               | Wt. %  | Cu. % | Cu. % |            |
| Heads.....    | 100.   | 3.99  | 100.0 |            |
| 1st Cone..... | 10.3   | 25.08 | 64.7  |            |
| 2nd Cone..... | 4.0    | 14.97 | 15.0  |            |
| 3rd Cone..... | 5.1    | 9.70  | 12.4  |            |
| Tails.....    | 80.6   | 0.35  | 7.9   |            |

*Example 7.*—Bwana M'Kubwa ore ground to pass 65 mesh was made into a pulp with water and agitated for one minute with 0.32

pounds of pine oil, per ton of ore, and then a froth concentrate separated for three minutes. There was then further added 4 pounds of thio-phenol, 0.8 pounds of steam distilled pine oil, both per ton of ore, and the pulp agitated for one minute and then a second froth concentrate separated for three minutes. There was then further added 4 pounds of thio-phenol per ton of ore, the pulp agitated for one minute, and then a third froth separated for three minutes. The results are shown in the following table:

|               | Assays |       |       | Recoveries |
|---------------|--------|-------|-------|------------|
|               | Wt. %  | Cu. % | Cu. % |            |
| Heads.....    | 100.   | 4.08  | 100.  |            |
| 1st Cone..... | 20.5   | 6.71  | 33.7  | 85         |
| 2nd Cone..... | 9.6    | 24.56 | 57.8  |            |
| 3rd Cone..... | 7.4    | 3.61  | 6.5   |            |
| Tails.....    | 62.5   | 0.13  | 2.0   |            |

*Example 8.*—In another test 0.30 pounds of cresol and 4 pounds of thiophenol, both per ton of ore, were added together to a pulp of the same ore to form a first froth, instead of the successive addition of pine oil and thiophenol. By this procedure a first concentrate was obtained containing 17.85% copper and representing 85.3% of the copper in the ore.

*Example 9.*—Bwana M'Kubwa ore ground to pass 65 mesh was made into a pulp with water and agitated in a subaeration testing machine for one minute with 0.32 pounds of steam distilled pine oil, and then a first froth separated for three minutes. There was further added 4 pounds of potassium ethyl mercaptide per ton of ore, the pulp agitated for one minute, and then a second froth separated for three minutes. There was further added 4 pounds of potassium ethyl mercaptide per ton of ore, the pulp agitated for one minute, and then a third froth separated for three minutes. For comparison the same procedure was followed for a fourth and fifth froths, adding potassium xanthate, however, instead of the mercaptide. The results are shown in the following table, from which it will be seen that the mercaptide produced a hitherto unequalled recovery of copper from this ore, although not as good a recovery as in other examples of this specification:

|               | Assays |       |       | Recoveries |
|---------------|--------|-------|-------|------------|
|               | Wt. %  | Cu. % | Cu. % |            |
| Heads.....    | 100.   | 3.81  | 100.  |            |
| 1st Conc..... | 19.6   | 5.79  | 29.0  |            |
| 2nd Conc..... | 12.2   | 13.0  | 40.9  |            |
| 3rd Conc..... | 11.4   | 5.79  | 8.1   |            |
| 4th Conc..... | 3.2    | 6.5   | 5.4   |            |
| 5th Conc..... | 1.8    | 16.15 | 7.5   |            |
| Tails.....    | 58.0   | 0.67  | 8.6   | 130        |

Para-thio-cresol when dissolved in acetone and then added to an ore pulp in large amounts, yielded, with cresol as a mineral-frothing agent, the same kind of froth as did 5 large amounts of xanthate. When dissolved in caustic soda solution and then added in large amounts to an ore pulp or copper carbonate ore, with pine oil as a mineral-frothing agent, it produced a froth like that characteristic of large amounts of a xanthate. 10

Thio-beta-naphthol when dissolved in alcohol and then added in large amount to a copper carbonate ore pulp and agitated with a mineral-frothing agent and with silicate of 15 soda, yielded a dirty froth which, however, showed considerable concentration. Without the silicate of soda there was no useful result. Neither was any useful result obtained when the thio-beta-naphthol was added dry 20 to a carbonate of copper ore pulp containing a mineral-frothing agent or when dissolved in toluene or in caustic soda solution and then added.

Mercapto-benzo-thiazole dissolved in acetone yielded a dirty mineral-bearing froth 25 showing considerable concentration when added in acetone solution to a carbonate of copper ore pulp containing a mineral-frothing agent and silicate of soda and then agitating 30 ed. Better results were obtained with a de-slimed ore pulp. It yielded no useful result when added in caustic soda solution under similar conditions.

Having described certain embodiments of 35 the invention, what is claimed is:

1. The process of concentrating ores which consists in agitating a pulp of an ore containing a relatively large fraction of its metal values in carbonate form, under such conditions that a froth bearing such carbonate is produced substantially dependent upon the presence both of an organic mineral-frothing agent and an amount of the order of not less than a pound per ton of ore of an organic sulphhydric compound adapted to float such carbonate, to cause the flotation of such carbonate and of a relatively small proportion of the froth.

50 2. The process of concentrating ores which consists in agitating a pulp of an ore containing a relatively large fraction of copper carbonate, under such conditions that a copper-carbonate-bearing froth is produced substantially dependent upon the presence both of an organic mineral-frothing agent and an amount of the order of not less than a pound per ton of ore of an organic sulphhydric compound adapted to float such carbonate, 55 to cause the flotation of such carbonate and of a relatively small proportion of the gangue; and separating the froth.

60 3. The process of concentrating ores which consists in agitating a pulp of an ore containing a relatively large fraction of its metal

values in carbonate form, under such conditions that a froth bearing such carbonate is produced substantially dependent upon the presence both of an organic mineral-frothing agent and an amount of the order of not less than a pound per ton of ore of a xanthate, to cause the flotation of such carbonate and of a relatively small proportion of the gangue; and separating the froth. 70

4. The process of concentrating ores which consists in agitating a pulp of an ore containing a relatively large fraction of its metal values in carbonate form, under such conditions that a froth bearing such carbonate is produced substantially dependent upon the presence both of an organic mineral-frothing agent and of about four pounds of an organic sulphhydric compound adapted to float such carbonate, to cause the flotation of such carbonate and of a relatively small proportion of the gangue; and separating the froth. 75

5. The process of concentrating ores which consists in agitating a pulp of an ore containing a relatively large fraction of copper carbonate, under such conditions that a copper carbonate-bearing froth is produced substantially dependent upon the presence both of an organic mineral-frothing agent and of about four pounds per ton of a xanthate, to cause the flotation of such carbonate and of a relatively small proportion of the gangue; and separating the froth. 80

In testimony whereof, I have affixed my signature to this specification.

WILLIAM TROTTER. 100

105

110

115

120

125

130